

# UNITED STATES PATENT OFFICE.

FRIEDRICH OTTO GRIPP, OF BREMEN, GERMANY.

## PROCESS FOR MANUFACTURE OF BRIQUETS.

1,016,939.

Specification of Letters Patent.

Patented Feb. 13, 1912.

No Drawing.

Application filed May 18, 1911. Serial No. 628,033.

To all whom it may concern:

Be it known that I, FRIEDRICH OTTO GRIPP, a subject of the German Emperor, residing at Albersstrasse 6, Bremen, Germany, have 5 invented a certain new and useful Process for Manufacture of Briquets, of which the following is a specification.

The present invention has for its object a process for the manufacture of briquets from 10 substances which will not bind under pressure alone, such as coke-burning coals, ore, or coke, by means of a binding medium which becomes fluid when hot.

In briquetting substances of this kind, in 15 order to economize as much as possible in the costly binding material, they have hitherto generally been heated either by direct exposure to heat or by steam or the like and in some cases the briquets themselves 20 have been exposed to special treatment in hot and cold chambers after they have been compressed. All these methods are relatively costly because the heating of the whole of the material requires very considerable 25 quantities of heat. On the other hand the pressure reservoirs and hot and cold chambers that are necessary for these known processes are relatively expensive owing to their large dimensions and the transportation of 30 the material to and from the various places of treatment is also very onerous owing to the large quantities that have to be dealt with. A process has also been proposed in 35 which the mass of fuel to be briquetted remains cold. This process, however, entails the employment of large quantities of binding media which liquefy under heat so that the process is unprofitable and furthermore the employment of hydraulic binding ma- 40 terial is necessary to supplement the action of the liquefying binding agent. These hydraulic binding media constitute an undesirable addition because they increase the quantity of slag and ash and in point of fact 45 the large quantity of liquefying binding material necessary for this known process exerts a prejudicial effect because in the furnace the briquets retain their form with greater difficulty in proportion as they con- 50 tain large quantities of resin, pitch or the like, because the high percentage of binding medium liquefying under heat causes a disintegration of the briquets at furnace or blast heat and the large generation of gas

from the binding material when heated also 55 facilitates the disintegration of the briquets.

In accordance with the present invention the defects of the known processes are obviated in the following manner. In the first place the binding medium liquefying 60 under heat is added to approximately three times the quantity of coking coal a quantity of water approximately equivalent to the binding medium is distributed throughout the coking coal, thus constituting an auxiliary 65 mass which is then employed as a combining medium for the close burning crude mass, by which means it is possible to manufacture briquets by cold pressing which contain only about 4% of binding medium. 70

In forming the auxiliary mass approximately 60 parts of coking coal in a dry state are finely ground and then mixed with 20 parts of water at any desired temperature, cold water being usually simplest and 75 most convenient. Approximately 20 parts of binding medium liquefying under heat are then added to the resultant mass and the whole is carefully mixed. When the binding medium is added and the mixing effected 80 the entire mass swells, the binding medium becoming extremely finely distributed throughout the mass as a whole. About 20% of the auxiliary mass thus constituted is then added to the crude mass composed 85 of the materials first mentioned, whereupon the briquetting takes place without special heating of the material under high pressure amounting to some 400 atmospheres. As the auxiliary mass contains only about 20% 90 of binding material the total proportion of binding material contained in the finished briquet is only about 4%.

The binding material is suitably selected for the use to which the briquet is to be put. 95 In the case of briquets for industrial purposes, when the smell is immaterial, the binding material may be pitch or pitch with admixtures of tar, naphtha and masut. For briquets for household burning the binding 100 material may consist of two parts of ordinary commercial resin and one part of mineral oil.

The auxiliary mass must not be manufactured separately; at the contrary by suitably positioning and regulating the supply pipes or supply channels of the mixing machine in which the whole mass is mixed, it 105

may be attained that the auxiliary mass is continuously formed at the point where the coking coal the water and the binding material is introduced.

5      Briquets made according to this process are weatherproof in that they do not require to be coated with an insulating material, and they are also fireproof to the extent that they retain their form under the heat and  
10     blast of stoves. The binder is of such a character that there is no generation of gases which would cause the briquet to be destroyed at once. The binding agent employed is intimately mixed with the mass by  
15     the method described of mixing the binder while hot with the coking coal in the presence of water. The briquets made according to this process are weatherproof, as they contain nothing affected by moisture, and  
20     by the use of the high pressure required by the binding agent used, the porosity of the briquets is very much diminished, if not wholly removed. The briquets also resist the action of the fire to a maximum degree,  
25     as they contain nothing developing vapor or

gases under the influence of the heat, a serious objection in processes of making briquets heretofore known.

What I claim and desire to secure by Letters Patent of the United States is:—

30     A process for making briquets from substances not binding under pressure alone, (such as close-burning coal or coke) consisting in first mixing a quantity of the coking coal with water, then adding a binding material liquefied under heat in the proportion approximately of four times the mixture of coking coal and water and one part of the binding material, and then adding this auxiliary mass to the mass of material 35 of which the briquets are to be made, and then pressing the commingled masses into the form of briquets, substantially as described.

35     In testimony whereof I affix my signature 40 in presence of two witnesses.

FRIEDRICH OTTO GRIPP.

Witnesses:

HENRY HASPER,  
WOLDEMAR HAUPT.